

# United States Patent Office.

JAMES D. WHELPLEY AND JACOB J. STORER, OF BOSTON, MASSACHUSETTS.

*Letters Patent No. 95,295, dated September 28, 1869; antedated September 16, 1869.*

## IMPROVED PROCESS OF OBTAINING WROUGHT-IRON DIRECTLY FROM THE ORE.

The Schedule referred to in these Letters Patent and making part of the same.

*To all whom it may concern:*

Be it known that we, JAMES D. WHELPLEY and JACOB J. STORER, of Boston, in the county of Suffolk, and State of Massachusetts, have invented a new and useful Process for Obtaining Wrought-Iron Directly from the Ore; and we do hereby declare that the following is a full, clear, and exact description of the construction and operation of the same.

The leading features of our process for the manufacture of iron and steel are based upon the principles of minute pulverization of the ore to be reduced, and the employment of the machine blow-pipe patented to us, March 13, 1866.

When the blast, conveying particles of carbon, floated, as dust, in its air-current, is employed, and is directed along a heated flue, or through an oven, by regulating and proportioning the supply of air and coal properly to each other, we obtain a carbonizing or reducing-flame—a neutral flame, or one which does not oxidize or quickly carbonize, and which may readily be made to give a welding-heat—or an oxidizing-flame, at the will of the operator, and thus the machine blow-pipe, or carbon-blast, gives us full control of all reasonable temperatures, and of all degrees of carburization and deoxidation of ores and metals required in metallurgy.

In the selection and employment of fluxes, the metallurgist will always be guided by an analysis of the ore to be worked, and the added ingredients must be adjusted by the operator to supplement the impurities to be eliminated from the ores. To form slags that shall fuse at low temperature, and demand the smallest possible sacrifice of iron in their formation, we prefer to so adjust the ingredients forming the slag, by observation of the character of the impurities of the ore, and selection of the fluxes to be added, that complex, and not simple slags shall be formed. The ingredients of the fluxes added are such as are well known to metallurgists; carbonates and oxides, particularly, of the alkalies and alkaline earths; silica, if the ore be deficient in that; chlorides and fluorides of the earths and alkalies, to reduce the point of fusion, and more effectively eliminate sulphur; (oxides of the less noble metals, such as lead and zinc, may often be used to advantage in eliminating sulphur and its congeners;) nitrates or chlorates of the alkalies and earths, to oxidize oxidizable impurities. These all are indicated by ordinary metallurgic knowledge for use as fluxes, and will be selected by the operator with a due regard to economy and efficiency.

The treatment of an ore by our process consists of three manipulations:

### *Manipulation I.*

The ore is first pulverized to dust. This is best done by means of our patented mills. In the process of pulverizing, suitable reagents, also finely pulverized,

are mingled with it, to act as fluxes, and eliminate the impurities of the ore.

This fine pulverization and intimate mixture of the ore and reagents give, measurably, the economies of time, fuel, and labor, which characterize the process, and exert a control over the purity and character of the iron and steel produced.

### *Manipulation II.*

The finely-pulverized material is spread (to the depth of a few inches) on the floor of a reverberatory furnace, and is there exposed, with frequent stirring, to the flame of the machine blow-pipe. The furnace should, preferably, have a hearth of wrought-iron. The flame should be oxidizing until the material has been raised to a bright red. At this point, the volatile impurities are eliminated or neutralized, and the sulphur and phosphorus do not after this appear in the iron in injurious excess. The oxidizing-flame is then changed to the carbonizing or reducing-flame, and the operation continued without raising the temperature. If the ore be constantly stirred, about half an hours' working in the furnace will bring the charge "to nature," or reduce the iron.

Here the second manipulation is varied, if we desire to produce steel from what it would be if we wish only to get blooms. If steel is to be produced, the reducing or carbonizing-flame is continued, and the iron rapidly absorbs carbon.

The degree of carbonization is determined by the length of exposure to the carbon-blast. An hour in the furnace is generally sufficient to produce the steel-sponge. Further exposure would give an iron of the character of cast-iron.

The heat on the hearth of the furnace should never reach the full melting-point of cast-iron.

The conclusion of this manipulation, whether iron or steel be sought, consists in raising the temperature, by applying the neutral flame, so as to fuse the fluxes, when the iron may be balled up, as in the process of puddling; or, if steel-sponge be the result, it is withdrawn from the furnace enveloped in slag, each particle being, as it were, jacketed with the slag formed of the earthy impurities and added fluxes.

The important point in this manipulation seems to us to be, that the ore is deoxidized, brought to nature, and carburetted to any desired degree, at a temperature below the fusing-point of the fluxes, and that when the fluxes are fused, a very small percentage of oxide of iron is present to be sacrificed by combining with the slag.

Alloys of iron, with manganese, tungsten, chromium, and the like, can best be obtained by mixing their oxides, salts, or carburets, with the ore in the first manipulation.

A small quantity of coal and carbonate of lime, pul-

verized with the ore in the first manipulation, generates carbonic oxide in the mass during the second, and the charge is thus rendered porous, and more permeable to the carbon-blast, so that the work of reduction is somewhat more rapid and complete.

By sampling the charge in the furnace, the progress of the work is ascertained, and the process may be stopped at any required stage of reduction or carburation.

*Manipulation III.*

In case wrought-iron is the desired product, the balls formed in the furnace would be squeezed, hammered, rolled, piled, and otherwise treated, as is usual in the making of wrought-iron from puddlers' balls; or the ore, slightly carbonized, may be removed to a proper puddling-furnace, and be there decarbonized and worked, as required; but, if steel or cast-iron be the desired product, the sponge is melted in crucibles, or treated in the hollow hearth of a reverberatory fur-

nace, lined with refractory material, and having the machine blow-pipe attached.

A high heat is required to melt the steel, and separate it from slag, which will float, and may be drawn off at will. When melted, it will be sampled and tested, and, if too highly carbonized, reduced, by adding slightly-carbonized sponge, wrought-iron, iron oxide, or other oxidizing-substances. If of too low a grade, its grade may be raised by adding highly-carbonized sponge, cast-iron, or carbon. We prefer, however, to control the degree of carbonization by the flame of the blow-pipe attached to the melting-furnace.

We claim the process of obtaining wrought-iron and its alloys directly from the ore, in the manner, and with the manipulations, and order of manipulation, substantially as described.

JAMES D. WHELPLEY.

Witnesses: JACOB J. STORER.

THOS. WM. CLARKE,

FRED. W. LONGLEY.